

## UNITED STATES PATENT OFFICE

WILLIAM A. DOUGLASS, OF PENNS GROVE, NEW JERSEY, ASSIGNOR TO E. I. DU PONT DE NEMOURS & COMPANY, OF WILMINGTON, DELAWARE, A CORPORATION OF DELAWARE

## PROCESS OF CONCENTRATING ORES AND MINERALS BY FLOTATION

No Drawing.

Application filed July 9, 1928. Serial No. 291,494.

This invention relates to the concentration of certain ores and minerals by flotation and comprises more particularly the concentration of such ores and minerals by means of a new class of organic flotation reagents.

This application is in the nature of a continuation in part of an application filed by the same inventor February 25, 1925, Serial No. 11,589.

10 It has been shown by Sayre in U. S. P. #1,512,139 that the heavy metal salts of xanthic acid are admirable flotation agents in a non-acid or alkaline pulp. Such xanthates are claimed to have a marked selective 15 action on sulfide minerals, as distinguished from gangue minerals and cause the sulfide minerals to float readily with an attendant high recovery of metal values. Both the heavy metal and alkali metal salts of xanthic 20 acid while of unquestioned value as flotation agents are open to certain objections in respect to purity and stability.

One object of my invention is to provide a class of flotation agents which not only 25 possess the good flotation properties resulting from the presence of the chemically reactive xanthic acid group, but which are chemically stable, and have flotation properties equal to or better than those possessed 30 by the heavy metal salts of xanthic acid. Moreover, I have found it possible to produce compounds of this type in a very pure state.

I have discovered that the compounds obtainable by treating a metal salt of xanthic acid or of an analogous sulfur or O containing acid with cyanogen halide as distinguished from metal xanthates, constitute excellent flotation agents and possess the desirable properties specified above.

These new organic flotation agents have in general a molecular structure indicated by the formula



45 where R represents an alkyl group, both radicals Y' represent the same element of the group consisting of O and S, both radicals Y''' represent the same element of the group

consisting of O and S, and Y''' represents either O or S.

The aliphatic derivatives of xanthic acid constitute a class of this broad group of compounds which has been found to contain compounds particularly well adapted for use in flotation and my invention will be described hereinafter with more particular reference thereto, as the preferred embodiment.

The flotation agents of this class of compounds have the general line formula:



where R and R' represent the same or different hydrocarbon radicals, preferably alkyl radicals. This class includes the corresponding symmetrical xanthyl monosulfides (that is, xanthic acid anhydrides) such as di-ethyl-xanthyl monosulfide,  $C_2H_5OCSSCSOC_2H_5$ .

As examples of other xanthic derivatives adapted for use as flotation agents there may be mentioned:

Di-methyl-xanthic anhydride,  
Di-propyl-xanthic anhydride,  
Di-butyl-xanthic anhydride,  
Di-amyl-xanthic anhydride,  
Ethyl-butyl-xanthic anhydride,  
Methyl-ethyl-xanthic anhydride,  
Methyl-butyl-xanthic anhydride.

Flotation tests with ethyl-xanthic anhydride, carried out on Inspiration ore gave the following results in comparison with potassium xanthate.

|                                               | Potassium xanthate | Ethyl xanthic anhydride | 85 |
|-----------------------------------------------|--------------------|-------------------------|----|
| Lbs. reagent/ton ore.....                     | 0.004              | 0.004                   |    |
| Per cent copper in heads.....                 | 1.03               | 1.03                    |    |
| Per cent copper in rougher tailings.....      | 0.41               | 0.32                    |    |
| Per cent copper recovered in concentrate..... | 62.2               | 70.4                    | 90 |
| Per cent copper in rougher concentrate.....   | 12.50              | 14.00                   |    |

The symmetrical anhydrides, in general, may be prepared by treating the appropriate metal xanthate or metal salt of an analogous acid with a cyanogen halide as illustrated by the equation:



50 The unsymmetrical monosulfides may be 100

similarly prepared by treating a mixture of the appropriate alkyl xanthates with cyanogen halide.

The xanthic anhydrides may also be prepared as a by-product by the action of the corresponding alkyl chlor formate and potassium alkyl xanthate. Ethyl xanthic anhydride, for example, may be prepared by the action of ethyl chlor formate on potassium ethyl xanthate. This crude product may be purified by separating the xanthic anhydride by cooling to  $-5^{\circ}\text{C}$ . The resulting product may be further purified, if desired, by recrystallization from absolute alcohol. A purified product so obtained contained 45.6% sulfur.

Welde (J. fur. Prak. Chemie (2) 15, (1877), p. 45) assumes that xanthic anhydride is formed by this method according to the following equation:



The various crude products prepared by the methods indicated above may contain in addition to the major products other xanthic compounds. Such products, however, may be employed in their crude state and may be introduced into the pulp or ore at any time prior to the flotation operation.

While the xanthate compounds have been employed above for the purposes of illustration, it will be understood from what has been said above by those skilled in the art that sulfur atoms may be replaced by oxygen or vice versa either in the double bonded positions or the single bonded positions. It is obvious that a large number of permutations and combinations is possible. The resulting compounds may be of any of the types indicated in the table below.



where  $\text{R}$  and  $\text{R}'$  represent the same or different alkyl radicals.

Although the new flotation agents have been found to be effective to a certain extent in an acid pulp, much better results are generally obtained by operating with a non-acid pulp, that is, one which has been rendered neutral or alkaline, preferably with lime. A frothing agent, as for example, terpineol, is also, ordinarily necessary since the new flotation agents have little, if any, frothing power.

I claim:

1. In the process of concentrating ores by flotation, the step which comprises subjecting the ore in the form of a pulp to a

froth flotation operation in the presence of the product resulting from the reaction between a compound of the group consisting of metal xanthates and analogues thereof and a cyanogen halide.

2. In the process of concentrating ores by flotation, the step which comprises subjecting the ore in the form of a pulp to a froth flotation operation in the presence of a compound having the general formula:



where  $\text{R}$  and  $\text{R}'$  represent alkyl groups, both radicals  $\text{Y}'$  represent the same element of the group consisting of O and S, both radicals  $\text{Y}'''$  represent the same element of the group consisting of O and S and  $\text{Y}'''$  represents an element of the group consisting of O and S.

3. In the process of concentrating ores by flotation, the step which comprises subjecting the ore in the form of a pulp to a froth flotation operation in the presence of a compound having the general formula:



where  $\text{R}$  and  $\text{R}'$  represent alkyl groups, both radicals  $\text{Y}'$  represent the same element of the group consisting of O and S, both radicals  $\text{Y}''$  represent the same element of the group consisting of O and S and  $\text{Y}'''$  represents an element of the group consisting of O and S but  $\text{Y}'$ ,  $\text{Y}''$  and  $\text{Y}'''$  do not all represent the same element of the group consisting of O and S.

4. In the process of concentrating ores by flotation, the step which comprises subjecting the ore in the form of a pulp to a froth flotation operation in the presence of a compound having the general formula:



where  $\text{R}$  and  $\text{R}'$  represent alkyl groups,  $\text{Y}'$  represents O, both radicals  $\text{Y}''$  represent the same element of the group consisting of O and S and  $\text{Y}'''$  represents an element of the group consisting of O and S.

5. In the process of concentrating ores by flotation, the step which comprises subjecting the ore in the form of a pulp to a froth flotation operation in the presence of a compound having the general formula:



where  $\text{R}$  and  $\text{R}'$  represent alkyl groups,  $\text{Y}'$  represents O,  $\text{Y}''$  represents S and  $\text{Y}'''$  represents an element of the group consisting of O and S.

6. In the process of concentrating ores by flotation, the step which comprises subjecting the ore in the form of a pulp to a froth

flotation operation in the presence of a compound having the formula:



5 where R and R' represent hydrocarbon radicals.

7. In the process of concentrating ores by flotation, the step which comprises subjecting the ore in the form of a pulp to a froth flotation operation in the presence of a symmetrical xanthic anhydride.

10 8. The improvement in the concentration of minerals by froth flotation which comprises subjecting the mineral in the form of 15 a pulp to a froth flotation operation in the presence of a xanthic anhydride.

9. The improvement in the concentration 20 of minerals by froth flotation which comprises subjecting the mineral in the form of a pulp to a froth flotation operation in the presence of an alkyl xanthic anhydride.

25 10. The improvement in the concentration of minerals by froth flotation which comprises subjecting the mineral in the form of a pulp to a froth flotation operation in the presence of an ethyl xanthic anhydride.

30 11. In the process of concentrating ores by flotation, the step which comprises subjecting the ore in the form of a pulp to a froth flotation operation in the presence of the product resulting from the reaction between an alkali metal xanthate and a cyanogen halide.

35 12. In the process of concentrating ores by flotation, the step which comprises subjecting the ore in the form of a pulp to a froth flotation operation in the presence of the product resulting from the reaction between an alkali metal xanthate and cyanogen 40 chloride.

45 13. In the process of concentrating ores by flotation, the step which comprises subjecting the ore in the form of a pulp to a froth flotation operation in the presence of the product resulting from the reaction between sodium ethyl xanthate and a cyanogen halide.

50 14. In the process of concentrating ores by flotation, the step which comprises subjecting the ore in the form of a pulp to a froth flotation operation in the presence of the product resulting from the reaction between sodium ethyl-xanthate and cyanogen chloride.

55 15. The improvement in the concentration of minerals by froth flotation which comprises subjecting the mineral in the form of a pulp to a froth flotation operation in the presence of diethyl-xanthic anhydride.

60 16. The improvement in the concentration of minerals by froth flotation which comprises subjecting the mineral in the form of a pulp to a froth flotation operation in the presence of dimethyl-xanthic anhydride.

65 17. The improvement in the concentration of minerals by froth flotation which comprises subjecting the mineral in the form of

a pulp to a froth flotation operation in the presence of dibutyl-xanthic anhydride.

18. The improvement in the concentration of minerals by froth flotation which comprises subjecting the mineral in the form of 70 a pulp to a froth flotation operation in the presence of a xanthic anhydride from the group consisting of dimethyl-xanthic anhydride, dipropyl-xanthic anhydride, dibutyl-xanthic anhydride, diamyl-xanthic anhydride, ethyl-butyl-xanthic anhydride, methyl-ethyl-xanthic anhydride and methyl-butyl-xanthic anhydride. 75

In testimony whereof, I affix my signature.

WILLIAM A. DOUGLASS. 80